



US011181843B2

(12) **United States Patent**  
Takeuchi et al.

(10) **Patent No.:** US 11,181,843 B2  
(45) **Date of Patent:** Nov. 23, 2021

(54) **ELECTROSTATIC-IMAGE DEVELOPING TONER, ELECTROSTATIC-IMAGE DEVELOPER, TONER CARTRIDGE, PROCESS CARTRIDGE, IMAGE FORMING APPARATUS, AND IMAGE FORMING METHOD**

(71) **Applicant:** FUJIFILM Business Innovation Corp., Tokyo (JP)

(72) **Inventors:** Sakiko Takeuchi, Kanagawa (JP); Daisuke Noguchi, Kanagawa (JP); Yuka Yamagishi, Kanagawa (JP); Yutaka Saito, Kanagawa (JP); Kazuhiko Nakamura, Kanagawa (JP)

(73) **Assignee:** FUJIFILM Business Innovation Corp., Tokyo (JP)

(\*) **Notice:** Subject to any disclaimer, the term of this patent is extended or adjusted under 35 U.S.C. 154(b) by 0 days.

(21) **Appl. No.:** 16/841,689

(22) **Filed:** Apr. 7, 2020

(65) **Prior Publication Data**

US 2021/0088923 A1 Mar. 25, 2021

(30) **Foreign Application Priority Data**

Sep. 19, 2019 (JP) ..... JP2019-170505

(51) **Int. Cl.**

*G03G 9/08* (2006.01)  
*G03G 9/097* (2006.01)  
*G03G 21/00* (2006.01)  
*G03G 15/08* (2006.01)  
*G03G 21/18* (2006.01)  
*G03G 9/113* (2006.01)

(52) **U.S. Cl.**  
CPC ..... *G03G 9/09708* (2013.01); *G03G 9/0819* (2013.01); *G03G 9/0821* (2013.01); *G03G 9/09725* (2013.01); *G03G 9/1138* (2013.01); *G03G 9/1139* (2013.01); *G03G 15/0865* (2013.01); *G03G 21/0011* (2013.01); *G03G 21/1814* (2013.01)

(58) **Field of Classification Search**  
CPC ..... G03G 9/09708; G03G 9/1138; G03G 9/1139; G03G 9/0819; G03G 9/0821  
USPC ..... 430/108.1  
See application file for complete search history.

(56) **References Cited**

U.S. PATENT DOCUMENTS

8,974,999 B1 \* 3/2015 Morales-Tirado ... G03G 9/0819  
430/123.51  
2005/0214668 A1 \* 9/2005 Miyakawa ..... G03G 9/09725  
430/108.7  
2008/0160440 A1 \* 7/2008 Nishikawa ..... G03G 9/1139  
430/108.6

FOREIGN PATENT DOCUMENTS

|    |            |         |
|----|------------|---------|
| JP | 2006317489 | 11/2006 |
| JP | 2009237274 | 10/2009 |

\* cited by examiner

*Primary Examiner* — Mark A Chapman

(74) **Attorney, Agent, or Firm:** JCIPRNET

(57) **ABSTRACT**

An electrostatic-image developing toner includes toner particles, layered compound particles, and a free oil. The mass ratio Ma/Mb of the content Ma of the layered compound particles to the content Mb of the free oil is 0.05 or more and 100 or less.

20 Claims, 2 Drawing Sheets



FIG. 1



FIG. 2



## 1

**ELECTROSTATIC-IMAGE DEVELOPING  
TONER, ELECTROSTATIC-IMAGE  
DEVELOPER, TONER CARTRIDGE,  
PROCESS CARTRIDGE, IMAGE FORMING  
APPARATUS, AND IMAGE FORMING  
METHOD**

**CROSS-REFERENCE TO RELATED  
APPLICATIONS**

This application is based on and claims priority under 35 USC 119 from Japanese Patent Application No. 2019-170505 filed Sep. 19, 2019.

**BACKGROUND**

(i) Technical Field

The present disclosure relates to an electrostatic-image developing toner, an electrostatic-image developer, a toner cartridge, a process cartridge, an image forming apparatus, and an image forming method.

(ii) Related Art

Japanese Laid Open Patent Application Publication No. 2006-317489 discloses a toner that includes toner base particles having an average circularity of 0.94 to 0.995 and a volume-average particle size of 3 to 9  $\mu\text{m}$  and melamine cyanurate powder particles having a volume-average particle size of 3 to 9  $\mu\text{m}$  which are deposited on the toner base particles such that the amount of the melamine cyanurate powder particles is 0.1 to 2.0 parts by weight relative to 100 parts by weight of the toner base particles.

Japanese Laid Open Patent Application Publication No. 2009-237274 discloses a positively chargeable toner that includes colored resin particles including a binder resin, a colorant, and a positively-charging control agent and melamine cyanurate particles having a number-average primary particle size of 0.05 to 1.5  $\mu\text{m}$  which are deposited on the colored resin particles such that the amount of the melamine cyanurate particles is 0.01 to 0.5 parts by weight relative to 100 parts by weight of the colored resin particles.

**SUMMARY**

Aspects of non-limiting embodiments of the present disclosure relate to an electrostatic-image developing toner that may reduce the formation of colored streaks which is caused as a result of a blade used for cleaning an image holding member becoming worn when an image is continuously formed in a high-temperature, high-humidity environment and the formation of colored streaks which is caused as a result of toner particles slipping through the portion at which an image holding member and the cleaning blade come into contact with each other when an image is continuously formed in a low-temperature, low-humidity environment, compared with an electrostatic-image developing toner that includes toner particles, layered compound particles, and a free oil, wherein the mass ratio Ma/Mb of the content Ma of the layered compound particles to the content Mb of the free oil is less than 0.05 or more than 100.

Aspects of certain non-limiting embodiments of the present disclosure address the above advantages and/or other advantages not described above. However, aspects of the non-limiting embodiments are not required to address the

## 2

advantages described above, and aspects of the non-limiting embodiments of the present disclosure may not address advantages described above.

According to an aspect of the present disclosure, there is provided an electrostatic-image developing toner including toner particles, layered compound particles, and a free oil. A mass ratio Ma/Mb of a content Ma of the layered compound particles to a content Mb of the free oil is 0.05 or more and 100 or less.

**10 BRIEF DESCRIPTION OF THE DRAWINGS**

An exemplary embodiment of the present disclosure will be described in detail based on the following figures, wherein:

15 FIG. 1 is a schematic diagram illustrating an example of an image forming apparatus according to an exemplary embodiment; and

20 FIG. 2 is a schematic diagram illustrating an example of a process cartridge according to an exemplary embodiment which is detachably attachable to an image forming apparatus.

**DETAILED DESCRIPTION**

25 An exemplary embodiment of the present disclosure is described below. The following description and Examples below are intended to be illustrative of the exemplary embodiment and not restrictive of the scope of the exemplary embodiment.

30 In the present disclosure, a numerical range expressed using “to” means the range specified by the minimum and maximum described before and after “to”, respectively.

In the present disclosure, when numerical ranges are described in a stepwise manner, the upper or lower limit of 35 a numerical range may be replaced with the upper or lower limit of another numerical range, respectively. In the present disclosure, the upper and lower limits of a numerical range may be replaced with the upper and lower limits described in Examples below.

40 The term “step” used herein refers not only to an individual step but also to a step that is not distinguishable from other steps but achieves the intended purpose of the step.

In the present disclosure, when an exemplary embodiment is described with reference to a drawing, the structure of the 45 exemplary embodiment is not limited to the structure illustrated in the drawing. The sizes of the members illustrated in the attached drawings are conceptual and do not limit the relative relationship among the sizes of the members.

Each of the components described in the present disclosure may include plural types of substances that correspond to the component. In the present disclosure, in the case where a composition includes plural substances that correspond to a component of the composition, the content of the component in the composition is the total content of the 50 plural substances in the composition unless otherwise specified.

In the present disclosure, the number of types of particles that correspond to a component may be two or more. In the case where a composition includes plural types of particles 55 that correspond to a component of the composition, the particle size of the component is the particle size of a mixture of the plural types of particles included in the composition unless otherwise specified.

In the present disclosure, an electrostatic-image developing toner may be referred to simply as “toner”, and an electrostatic-image developer may be referred to simply as “developer”.

## Electrostatic-Image Developing Toner

A toner according to the exemplary embodiment includes toner particles, layered compound particles, and a free oil. The mass ratio Ma/Mb of the content Ma of the layered compound particles to the content Mb of the free oil is 0.05 or more and 100 or less.

The toner according to the exemplary embodiment may reduce the formation of colored streaks which is caused as a result of a blade used for cleaning an image holding member becoming worn when an image is continuously formed in a high-temperature, high-humidity environment (e.g., at 28° C. and a relative humidity of 85%) and the formation of colored streaks which is caused as a result of toner particles slipping through the portion at which an image holding member and the cleaning blade come into contact with each other when an image is continuously formed in a low-temperature, low-humidity environment (e.g., at 10° C. and a relative humidity of 10%). The mechanisms for this are presumably as described below.

Toners that include layered compound particles, such as melamine cyanurate particles and boron nitride particles, used as an external additive are known. The layered compound particles are particles of a compound having a layered structure with an interlayer distance of the order of angstroms and are considered to produce a lubricating effect as a result of the layers becoming displaced with respect to one another. The layered compound particles deposited on the toner particles as an external additive serve as a lubricant at the portion at which an image holding member and the cleaning blade come into contact with each other.

Since the layered compound particles have relatively low moisture absorbency, the layered compound particles are resistant to degradation and likely to maintain the lubricating effect even under the condition where an image is formed in a high-temperature, high-humidity environment, that is, even under the condition where a voltage is applied to the layered compound particles on an image holding member in a high-temperature, high-humidity environment. However, if an image is continuously formed for a long period of time in a high-temperature, high-humidity environment, the lubricating effect of the layered compound particles may be reduced and, consequently, colored streaks may be formed as a result of the wearing of the cleaning blade.

While external additive particles accumulate at the portion at which the cleaning blade and an image holding member come into contact with each other to form sediments (i.e., "external additive dam"), the layered compound particles are less likely to form the external additive dam than other external additives. Therefore, if an image is continuously formed with a toner including the layered compound particles for a long period of time in a low-temperature, low-humidity environment, that is, under the condition where the likelihood of formation of the external additive dam is low, the external additive dam may become brittle and, consequently, colored streaks may be formed as a result of the slip-through of toner particles.

In order to address the above issues, in the exemplary embodiment, the toner includes a free oil in addition to the layered compound particles and the content of the free oil in the toner is limited to fall within an adequate range. This may enhance the resistance of the layered compound particles to degradation and increase the strength of the external additive dam.

Accordingly, the toner according to the exemplary embodiment may reduce the formation of colored streaks which is caused as a result of a blade used for cleaning an image holding member becoming worn when an image is

continuously formed in a high-temperature, high-humidity environment and the formation of colored streaks which is caused as a result of toner particles slipping through the portion at which an image holding member and the cleaning blade come into contact with each other when an image is continuously formed in a low-temperature, low-humidity environment.

In the toner according to the exemplary embodiment, the mass ratio Ma/Mb of the content Ma of the layered compound particles to the content Mb of the free oil is 0.05 or more and 100 or less.

If the ratio Ma/Mb is less than 0.05, that is, if the relative content of the free oil is excessively high, the free oil may reduce the lubricity of the layered compound particles and, consequently, colored streaks may be formed as a result of a blade used for cleaning an image holding member becoming worn when an image is continuously formed in a high-temperature, high-humidity environment.

If the ratio Ma/Mb is more than 100, that is, if the relative content of the free oil is excessively low, the strength of the external additive dam may fail to be increased to a sufficient degree and, consequently, colored streaks may be formed as a result of toner particles slipping through the portion at which an image holding member and the cleaning blade come into contact with each other when an image is continuously formed in a low-temperature, low-humidity environment.

From the above viewpoints, the ratio Ma/Mb is more preferably 0.2 or more and 100 or less and is further preferably 0.5 or more and 80 or less.

Details of the components, structure, and properties of the toner according to the exemplary embodiment are described below.

## 35 Toner Particles

The toner particles include, for example, a binder resin and may optionally include a colorant, a release agent, and other additives.

## Binder Resin

40 Examples of the binder resin include vinyl resins that are homopolymers of the following monomers or copolymers of two or more monomers selected from the following monomers: styrenes, such as styrene, para-chlorostyrene, and  $\alpha$ -methylstyrene; (meth)acrylates, such as methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, lauryl methacrylate, and 2-ethylhexyl methacrylate; ethylenically unsaturated nitriles, such as acrylonitrile and methacrylonitrile; vinyl ethers, such as vinyl methyl ether and vinyl isobutyl ether; vinyl ketones, such as vinyl methyl ketone, vinyl ethyl ketone, and vinyl isopropenyl ketone; and olefins, such as ethylene, propylene, and butadiene.

45 Examples of the binder resin further include non-vinyl resins, such as epoxy resins, polyester resins, polyurethane resins, polyamide resins, cellulose resins, polyether resins, and modified rosins; a mixture of the non-vinyl resin and the vinyl resin; and a graft polymer produced by polymerization of the vinyl monomer in the presence of the non-vinyl resin.

50 The above binder resins may be used alone or in combination of two or more.

The binder resin may be a polyester resin.

55 Examples of the polyester resin include amorphous polyester resins known in the related art. A crystalline polyester resin may be used as a polyester resin in combination with an amorphous polyester resin. In such a case, the content of the crystalline polyester resin in the binder resin may be 2%

by mass or more and 40% by mass or less and is preferably 2% by mass or more and 20% by mass or less.

The term "crystalline" resin used herein refers to a resin that, in thermal analysis using differential scanning calorimetry (DSC), exhibits a distinct endothermic peak instead of step-like endothermic change and specifically refers to a resin that exhibits an endothermic peak with a half-width of 10° C. or less at a heating rate of 10° C./min.

On the other hand, the term "amorphous" resin used herein refers to a resin that exhibits an endothermic peak with a half-width of more than 10° C., that exhibits step-like endothermic change, or that does not exhibit a distinct endothermic peak.

#### Amorphous Polyester Resin

Examples of the amorphous polyester resin include condensation polymers of a polyvalent carboxylic acid and a polyhydric alcohol. The amorphous polyester resin may be a commercially available one or a synthesized one.

Examples of the polyvalent carboxylic acid include aliphatic dicarboxylic acids, such as oxalic acid, malonic acid, maleic acid, fumaric acid, citraconic acid, itaconic acid, glutaconic acid, succinic acid, alkenyl succinic acid, adipic acid, and sebacic acid; alicyclic dicarboxylic acids, such as cyclohexanedicarboxylic acid; aromatic dicarboxylic acids, such as terephthalic acid, isophthalic acid, phthalic acid, and naphthalenedicarboxylic acid; anhydrides of these dicarboxylic acids; and lower (e.g., 1 to 5 carbon atoms) alkyl esters of these dicarboxylic acids. Among these dicarboxylic acids, for example, aromatic dicarboxylic acids may be used as a polyvalent carboxylic acid.

Trivalent or higher carboxylic acids having a crosslinked structure or a branched structure may be used as a polyvalent carboxylic acid in combination with the dicarboxylic acids. Examples of the trivalent or higher carboxylic acids include trimellitic acid, pyromellitic acid, anhydrides of these carboxylic acids, and lower (e.g., 1 to 5 carbon atoms) alkyl esters of these carboxylic acids.

The above polyvalent carboxylic acids may be used alone or in combination of two or more.

Examples of the polyhydric alcohol include aliphatic diols, such as ethylene glycol, diethylene glycol, triethylene glycol, propylene glycol, butanediol, hexanediol, and neopentyl glycol; alicyclic diols, such as cyclohexanediol, cyclohexanedimethanol, and hydrogenated bisphenol A; and aromatic diols, such as bisphenol A-ethylene oxide adduct and bisphenol A-propylene oxide adduct. Among these diols, for example, aromatic diols and alicyclic diols may be used as a polyhydric alcohol. In particular, aromatic diols may be used as a polyhydric alcohol.

Trihydric or higher alcohols having a crosslinked structure or a branched structure may be used as a polyhydric alcohol in combination with the diols. Examples of the trihydric or higher alcohols include glycerin, trimethylolpropane, and pentaerythritol.

The above polyhydric alcohols may be used alone or in combination of two or more.

The glass transition temperature  $T_g$  of the amorphous polyester resin is preferably 50° C. or more and 80° C. or less and is more preferably 50° C. or more and 65° C. or less.

The glass transition temperature is determined from a DSC curve obtained by differential scanning calorimetry (DSC). More specifically, the glass transition temperature is determined from the "extrapolated glass-transition-starting temperature" according to a method for determining glass transition temperature which is described in JIS K 7121: 1987 "Testing Methods for Transition Temperatures of Plastics".

The weight-average molecular weight  $M_w$  of the amorphous polyester resin is preferably 5,000 or more and 1,000,000 or less and is more preferably 7,000 or more and 500,000 or less.

The number-average molecular weight  $M_n$  of the amorphous polyester resin is preferably 2,000 or more and 100,000 or less.

The molecular weight distribution index  $M_w/M_n$  of the amorphous polyester resin is preferably 1.5 or more and 100 or less and is more preferably 2 or more and 60 or less.

The weight-average molecular weight and number-average molecular weight of the amorphous polyester resin are determined by gel permeation chromatography (GPC). Specifically, the molecular weights of the amorphous polyester resin are determined by GPC using a "HLC-8120GPC" produced by Tosoh Corporation as measuring equipment, a column "TSKgel SuperHM-M (15 cm)" produced by Tosoh Corporation, and a tetrahydrofuran (THF) solvent. The weight-average molecular weight and number-average molecular weight of the amorphous polyester resin are determined on the basis of the results of the measurement using a molecular-weight calibration curve based on monodisperse polystyrene standard samples.

The amorphous polyester resin may be produced by any suitable production method known in the related art. Specifically, the amorphous polyester resin may be produced by, for example, a method in which polymerization is performed at 180° C. or more and 230° C. or less, the pressure inside the reaction system is reduced as needed, and water and alcohols that are generated by condensation are removed.

In the case where the raw materials, that is, the monomers, are not dissolved in or miscible with each other at the reaction temperature, a solvent having a high boiling point may be used as a dissolution adjuvant in order to dissolve the raw materials. In such a case, the condensation polymerization reaction is performed while the dissolution adjuvant is distilled away. In the case where the monomers used in the copolymerization reaction have low miscibility with each other, a condensation reaction of the monomers with an acid or alcohol that is to undergo a polycondensation reaction with the monomers may be performed in advance and subsequently polycondensation of the resulting polymers with the other components may be performed.

#### Crystalline Polyester Resin

Examples of the crystalline polyester resin include condensation polymers of a polyvalent carboxylic acid and a polyhydric alcohol. The crystalline polyester resin may be commercially available one or a synthesized one.

In order to increase ease of forming a crystal structure, a condensation polymer prepared from linear aliphatic polymerizable monomers may be used as a crystalline polyester resin instead of a condensation polymer prepared from polymerizable monomers having an aromatic ring.

Examples of the polyvalent carboxylic acid include aliphatic dicarboxylic acids, such as oxalic acid, succinic acid, glutaric acid, adipic acid, suberic acid, azelaic acid, sebacic acid, 1,9-nonanedicarboxylic acid, 1,10-decanedicarboxylic acid, 1,12-dodecanedicarboxylic acid, 1,14-tetradecanedicarboxylic acid, and 1,18-octadecanedicarboxylic acid; aromatic dicarboxylic acids, such as dibasic acids (e.g., phthalic acid, isophthalic acid, terephthalic acid, and naphthalene-2,6-dicarboxylic acid); anhydrides of these dicarboxylic acids; and lower (e.g., 1 to 5 carbon atoms) alkyl esters of these dicarboxylic acids.

Trivalent or higher carboxylic acids having a crosslinked structure or a branched structure may be used as a polyvalent carboxylic acid in combination with the dicarboxylic acids.

Examples of the trivalent carboxylic acids include aromatic carboxylic acids, such as 1,2,3-benzenetricarboxylic acid, 1,2,4-benzenetricarboxylic acid, and 1,2,4-naphthalenetricharboxylic acid; anhydrides of these tricarboxylic acids; and lower (e.g., 1 to 5 carbon atoms) alkyl esters of these tricarboxylic acids.

Dicarboxylic acids including a sulfonic group and dicarboxylic acids including an ethylenic double bond may be used as a polyvalent carboxylic acid in combination with the above dicarboxylic acids.

The above polyvalent carboxylic acids may be used alone or in combination of two or more.

Examples of the polyhydric alcohol include aliphatic diols, such as linear aliphatic diols including a backbone having 7 to 20 carbon atoms. Examples of the aliphatic diols include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, 1,12-dodecanediol, 1,13-tridecanediol, 1,14-tetradecanediol, 1,18-octadecanediol, and 1,14-eicosanediol. Among these aliphatic diols, 1,8-octanediol, 1,9-nonanediol, and 1,10-decanediol may be used.

Trihydric or higher alcohols having a crosslinked structure or a branched structure may be used as a polyhydric alcohol in combination with the above diols. Examples of the trihydric or higher alcohols include glycerin, trimethylolethane, trimethylolpropane, and pentaerythritol.

The above polyhydric alcohols may be used alone or in combination of two or more.

The content of the aliphatic diols in the polyhydric alcohol may be 80 mol % or more and is preferably 90 mol % or more.

The melting temperature of the crystalline polyester resin is preferably 50° C. or more and 100° C. or less, is more preferably 55° C. or more and 90° C. or less, and is further preferably 60° C. or more and 85° C. or less.

The melting temperature of the crystalline polyester resin is determined from the "melting peak temperature" according to a method for determining melting temperature which is described in JIS K 7121:1987 "Testing Methods for Transition Temperatures of Plastics" using a DSC curve obtained by differential scanning calorimetry (DSC).

The crystalline polyester resin may have a weight-average molecular weight Mw of 6,000 or more and 35,000 or less.

The crystalline polyester resin may be produced by any suitable method known in the related art similarly to, for example, the amorphous polyester resin.

The content of the binder resin in the toner particles is preferably 40% by mass or more and 95% by mass or less, is more preferably 50% by mass or more and 90% by mass or less, and is further preferably 60% by mass or more and 85% by mass or less.

#### Colorant

Examples of the colorant include pigments, such as Carbon Black, Chrome Yellow, Hansa Yellow, Benzidine Yellow, Threne Yellow, Quinoline Yellow, Pigment Yellow, Permanent Orange GTR, Pyrazolone Orange, Vulcan Orange, Watching Red, Permanent Red, Brilliant Carmine 3B, Brilliant Carmine 6B, DuPont Oil Red, Pyrazolone Red, Lithol Red, Rhodamine B Lake, Lake Red C, Pigment Red, Rose Bengal, Aniline Blue, Ultramarine Blue, Calco Oil Blue, Methylene Blue Chloride, Phthalocyanine Blue, Pigment Blue, Phthalocyanine Green, and Malachite Green Oxalate; and dyes, such as acridine dyes, xanthene dyes, azo dyes, benzoquinone dyes, azine dyes, anthraquinone dyes, thioindigo dyes, dioxazine dyes, thiazine dyes, azomethine

dyes, indigo dyes, phthalocyanine dyes, aniline black dyes, polymethine dyes, triphenylmethane dyes, diphenylmethane dyes, and thiazole dyes.

The above colorants may be used alone or in combination of two or more.

The colorant may optionally be subjected to a surface treatment and may be used in combination with a dispersant. Plural types of colorants may be used in combination.

The content of the colorant in the toner particles is 10 preferably 1% by mass or more and 30% by mass or less and is more preferably 3% by mass or more and 15% by mass or less.

#### Release Agent

15 Examples of the release agent include, but are not limited to, hydrocarbon waxes; natural waxes, such as a carnauba wax, a rice bran wax, and a candelilla wax; synthetic or mineral-petroleum-derived waxes, such as a montan wax; and ester waxes, such as a fatty-acid ester wax and a montanate wax.

The melting temperature of the release agent is preferably 50° C. or more and 110° C. or less and is more preferably 60° C. or more and 100° C. or less.

The melting temperature of the release agent is determined from the "melting peak temperature" according to a method for determining melting temperature which is described in JIS K 7121:1987 "Testing Methods for Transition Temperatures of Plastics" using a DSC curve obtained by differential scanning calorimetry (DSC).

30 The content of the release agent in the toner particles is preferably 1% by mass or more and 20% by mass or less and is more preferably 5% by mass or more and 15% by mass or less.

#### Other Additives

35 Examples of the other additives include additives known in the related art, such as a magnetic substance, a charge-controlling agent, and an inorganic powder. These additives may be added to the toner particles as internal additives.

#### Properties, etc. of Toner Particles

40 The toner particles may have a single-layer structure or a "core-shell" structure constituted by a core (i.e., core particle) and a coating layer (i.e., shell layer) covering the core.

The core-shell structure of the toner particles may be constituted by, for example, a core including a binder resin and, as needed, other additives such as a colorant and a release agent and by a coating layer including the binder resin.

45 The volume-average diameter D50v of the toner particles is preferably 2 µm or more and 10 µm or less and is more preferably 4 µm or more and 8 µm or less.

The above-described average diameters and particle diameter distribution indices of the toner particles are measured using "COULTER Multisizer II" (produced by Beckman Coulter, Inc.) with an electrolyte "ISOTON-II" (produced by Beckman Coulter, Inc.) in the following manner.

50 A sample to be measured (0.5 mg or more and 50 mg or less) is added to 2 ml of a 5 mass %-aqueous solution of a surfactant (e.g., sodium alkylbenzene sulfonate) that serves as a dispersant. The resulting mixture is added to 100 ml or more and 150 ml or less of an electrolyte.

55 The resulting electrolyte containing the sample suspended therein is subjected to a dispersion treatment for 1 minute using an ultrasonic disperser, and the distribution of the diameters of particles having a diameter of 2 µm or more and 60 µm or less is measured using COULTER Multisizer II with an aperture having a diameter of 100 µm. The number of the particles sampled is 50,000.

The particle diameter distribution measured is divided into a number of particle diameter ranges (i.e., channels). For each range, in ascending order in terms of particle diameter, the cumulative volume and the cumulative number are calculated and plotted to draw cumulative distribution curves. Particle diameters at which the cumulative volume and the cumulative number reach 16%, are considered to be the volume particle diameter D16v and the number particle diameter D16p, respectively. Particle diameters at which the cumulative volume and the cumulative number reach 50% are considered to be the volume-average particle diameter D50v and the number-average particle diameter D50p, respectively. Particle diameters at which the cumulative volume and the cumulative number reach 84% are considered to be the volume particle diameter D84v and the number particle diameter D84p, respectively.

Using the volume particle diameters and number particle diameters measured, the volume grain size distribution index (GSDv) is calculated as  $(D84v/D16v)^{1/2}$  and the number grain size distribution index (GSDp) is calculated as  $(D84p/D16p)^{1/2}$ .

The toner particles preferably has an average circularity of 0.94 or more and 1.00 or less. The average circularity of the toner particles is more preferably 0.95 or more and 0.98 or less.

The average circularity of the toner particles is determined as [Equivalent circle perimeter]/[Perimeter] (i.e., [Perimeter of a circle having the same projection area as the particles]/[Perimeter of the projection image of the particles]). Specifically, the average circularity of the toner particles is determined by the following method.

The toner particles to be measured are sampled by suction so as to form a flat stream. A static image of the particles is taken by instantaneously flashing a strobe light. The image of the particles is analyzed with a flow particle image analyzer "FPIA-3000" produced by Sysmex Corporation. The number of samples used for determining the average circularity of the toner particles is 3,500.

In the case where the toner includes an external additive, the toner (i.e., the developer) to be measured is dispersed in water containing a surfactant and then subjected to an ultrasonic wave treatment in order to remove the external additive from the toner particles.

#### Layered Compound Particles

The layered compound particles are particles of a compound having a layered structure. Examples of the layered compound particles include melamine cyanurate particles, boron nitride particles, graphite fluoride particles, molybdenum disulfide particles, and mica particles.

The volume-average particle size of the layered compound particles may be 0.4  $\mu\text{m}$  or more and less than 3.0  $\mu\text{m}$  in order to reduce the formation of the colored streaks. When the volume-average particle size of the layered compound particles is 0.4  $\mu\text{m}$  or more, the layered compound particles may be resistant to degradation under the condition where a voltage is applied to the layered compound particles for a long period of time in a high-temperature, high-humidity environment. When the volume-average particle size of the layered compound particles is less than 3.0  $\mu\text{m}$ , the external additive dam may be readily formed.

From the above viewpoints, the volume-average particle size of the layered compound particles is more preferably 0.5  $\mu\text{m}$  or more and 2.5  $\mu\text{m}$  or less and is further preferably 0.5  $\mu\text{m}$  or more and 2.0  $\mu\text{m}$  or less. The volume-average particle size of the layered compound particles may be controlled by disintegration, classification, or a combination of disintegration and classification.

The volume-average particle size of the layered compound particles is determined by the following measuring method.

First, the layered compound particles are separated from the toner. The method for separating the layered compound particles from the toner is not limited. For example, an ultrasonic wave is applied to a dispersion liquid prepared by dispersing the toner particles in water containing a surfactant. The dispersion liquid is subjected to high-speed centrifugation to separate the toner particles, the layered compound particles, and the other external additive from one another by centrifugal force on the basis of specific gravity. The fraction containing the layered compound particles is extracted and dried to obtain layered compound particles.

The layered compound particles are added to an aqueous electrolyte solution (aqueous ISOTON solution). An ultrasonic wave is applied to the resulting mixture for 30 seconds or more in order to form a dispersion liquid. This dispersion liquid is used as a sample. The particle size of the layered compound particles is measured with a laser diffraction/scattering particle size distribution analyzer, such as "Microtrac MT3000II" produced by MicrotracBEL Corp. At least 3,000 layered compound particles are measured. The particle size at which the cumulative volume reaches 50% in a volume grain size distribution drawn in ascending order in terms of particle size is considered the volume-average particle size.

The content of the layered compound particles in the toner is preferably 0.01% by mass or more and 1.0% by mass or less, is more preferably 0.03% by mass or more and 0.8% by mass or less, and is further preferably 0.05% by mass or more and 0.6% by mass or less of the total amount of the toner in order to reduce the formation of the colored streaks.

#### Free Oil and Oil-Treated Particles

Examples of the free oil include a silicone oil, a paraffin oil, a fluorine oil, and a vegetable oil. The above free oils may be used alone or in combination of two or more. Among the above free oils, a silicone oil is preferable, and a dimethyl silicone oil is more preferable.

The content of the free oil in the toner is preferably 0.005% by mass or more and 0.2% by mass or less, is more preferably 0.01% by mass or more and 0.12% by mass or less, and is further preferably 0.02% by mass or more and 0.08% by mass or less of the total amount of the toner in order to reduce the formation of the colored streaks.

The content (%) of the free oil in the entire toner is determined by the following method.

Toner particles on which the external additive is deposited are dispersed in hexane such that the concentration of the toner in the resulting dispersion liquid is 5% by mass. An ultrasonic wave (power: 20 W, frequency: 20 kHz) is applied to the dispersion liquid for 20 minutes. The supernatant and the solid component are separated from each other by centrifugal force. The content (I) of the free oil in the entire toner is represented by the following formula.

$$\text{Free oil content (\%)} = (W_b - W_a) / W_b \times 100$$

where  $W_b$  is the mass of the toner used as a sample, and  $W_a$  is the mass of the solid component obtained by the centrifugal separation.

The free oil included in the toner may be an oil added to the toner or an oil released from the external additive deposited on the toner. For adding the free oil to the toner, particles treated with an oil may be deposited on the toner in order to make it easy to adjust the content of the free oil.

Examples of the particles treated with an oil include inorganic particles (e.g.,  $\text{SiO}_2$  particles,  $\text{TiO}_2$  particles,

## 11

$\text{Al}_2\text{O}_3$  particles,  $\text{CuO}$  particles,  $\text{ZnO}$  particles,  $\text{SnO}_2$  particles,  $\text{CeO}_2$  particles,  $\text{Fe}_2\text{O}_3$  particles,  $\text{MgO}$  particles,  $\text{BaO}$  particles,  $\text{CaO}$  particles,  $\text{K}_2\text{O}$  particles,  $\text{Na}_2\text{O}$  particles,  $\text{ZrO}_2$  particles,  $\text{CaO.SiO}_2$  particles,  $\text{K}_2\text{O}(\text{TiO}_2)_n$  particles,  $\text{Al}_2\text{O}_3.2\text{SiO}_2$  particles,  $\text{CaCO}_3$  particles,  $\text{MgCO}_3$  particles,  $\text{BaSO}_4$  particles, and  $\text{MgSO}_4$  particles) treated with an oil; resin particles (e.g., particles of polystyrene, polymethyl methacrylate, and a melamine resin) treated with an oil; and cleaning lubricant particles (e.g., particles of a metal salt of a higher fatty acid, such as zinc stearate, and particles of a fluorine-based high-molecular-weight compound) treated with an oil. The particles treated with an oil are preferably silica particles treated with an oil.

The oil treatment of the above particles is performed by, for example, dispersing the particles in an oil dissolved in an alcohol, removing the alcohol by distillation using an evaporator, and performing drying. Examples of the oil include a silicone oil, a paraffin oil, a fluorine oil, and a vegetable oil. Among the above oils, a silicone oil is preferable, and a dimethyl silicone oil is more preferable.

The content of the free oil in the oil-treated particles may be determined by the following method.

The oil-treated particles are dispersed in hexane such that the concentration of the oil-treated particles in the resulting dispersion liquid is 5% by mass. An ultrasonic wave (power: 20 W, frequency: 20 kHz) is applied to the dispersion liquid for 20 minutes. The supernatant and the solid component are separated from each other by centrifugal force. The content (mass %) of the free oil in the oil-treated particles is represented by the following formula.

$$\text{Free oil content(mass \%)} = (W_b - W_a) / W_b \times 100$$

where  $W_b$  is the mass of the oil-treated particles used as a sample, and  $W_a$  is the mass of the solid component obtained by the centrifugal separation.

The volume-average particle size of the oil-treated particles is preferably 40 nm or more and 300 nm or less, is more preferably 50 nm or more and 250 nm or less, and is further preferably 50 nm or more and 200 nm or less in order to reduce the formation of the colored streaks.

The content of the oil-treated particles in the toner is preferably 0.5% by mass or more and 4.0% by mass or less, is more preferably 0.5% by mass or more and 3.5% by mass or less, and is further preferably 0.7% by mass or more and 3.0% by mass or less of the total amount of the toner in order to reduce the formation of the colored streaks.

The mass ratio  $M_c/M_a$  of the content  $M_c$  of the oil-treated particles to the content  $M_a$  of the layered compound particles is preferably 0.5 or more and 400 or less, is more preferably 0.5 or more and 200 or less, and is further preferably 0.7 or more and 150 or less in order to reduce the formation of the colored streaks.

## Other External Additive

The toner according to the exemplary embodiment may include an external additive other than the oil-treated particles, that is, particles that are not treated with an oil. Examples of the particles that are not treated with an oil include inorganic particles, such as  $\text{SiO}_2$  particles,  $\text{TiO}_2$  particles,  $\text{Al}_2\text{O}_3$  particles,  $\text{CuO}$  particles,  $\text{ZnO}$  particles,  $\text{SnO}_2$  particles,  $\text{CeO}_2$  particles,  $\text{Fe}_2\text{O}_3$  particles,  $\text{MgO}$  particles,  $\text{BaO}$  particles,  $\text{CaO}$  particles,  $\text{K}_2\text{O}$  particles,  $\text{Na}_2\text{O}$  particles,  $\text{ZrO}_2$  particles,  $\text{CaO.SiO}_2$  particles,  $\text{K}_2\text{O}(\text{TiO}_2)_n$  particles,  $\text{Al}_2\text{O}_3.2\text{SiO}_2$  particles,  $\text{CaCO}_3$  particles,  $\text{MgCO}_3$  particles,  $\text{BaSO}_4$  particles, and  $\text{MgSO}_4$  particles; particles of a resin, such as polystyrene, polymethyl methacrylate, or a melamine resin; and particles of a cleaning lubricant, such as a metal salt of a higher fatty acid (e.g., zinc stearate) or a

## 12

fluorine-based high-molecular-weight compound. The above particles may be surface-treated with a hydrophobizing agent other than an oil, such as a coupling agent.

In the case where toner according to the exemplary embodiment includes the particles that are not treated with an oil, the total amount of the particles that are not treated with an oil which are used as an external additive is preferably 0.01% by mass or more and 5% by mass or less and is more preferably 0.01% by mass or more and 2.0% by mass or less of the amount of the toner particles.

## Method for Producing Toner

The toner according to the exemplary embodiment is produced by, after the preparation of the toner particles, depositing an external additive on the surfaces of the toner particles.

The toner particles may be prepared by any dry process, such as knead pulverization, or any wet process, such as aggregation coalescence, suspension polymerization, or dissolution suspension. However, a method for preparing the toner particles is not limited thereto, and any suitable method known in the related art may be used. Among these methods, aggregation coalescence may be used in order to prepare the toner particles.

Specifically, in the case where, for example, aggregation coalescence is used in order to prepare the toner particles, the toner particles are prepared by the following steps:

preparing a resin particle dispersion liquid in which resin particles serving as a binder resin are dispersed (i.e., resin particle dispersion liquid preparation step);

causing the resin particles (and, as needed, other particles) to aggregate together in the resin particle dispersion liquid (or in the resin particle dispersion liquid mixed with another particle dispersion liquid as needed) in order to form aggregated particles (i.e., aggregated particle formation step);

and heating the resulting aggregated particle dispersion liquid in which the aggregated particles are dispersed in order to cause fusion and coalescence of the aggregated particles to occur and thereby form toner particles (fusion-coalescence step).

Each of the above steps is described below in detail.

Hereinafter, a method for preparing toner particles including a colorant and a release agent is described. However, it should be noted that the colorant and the release agent are optional. It is needless to say that additives other than a colorant and a release agent may be used.

## Resin Particle Dispersion Liquid Preparation Step

In addition to a resin particle dispersion liquid in which resin particles serving as a binder resin is dispersed, for example, a colorant particle dispersion liquid in which colorant particles are dispersed and a release-agent particle dispersion liquid in which release-agent particles are dispersed are prepared.

The resin particle dispersion liquid is prepared by, for example, dispersing resin particles in a dispersion medium using a surfactant.

Examples of the dispersion medium used for preparing the resin particle dispersion liquid include aqueous media.

Examples of the aqueous media include water, such as distilled water and ion-exchange water; and alcohols. These aqueous media may be used alone or in combination of two or more.

Examples of the surfactant include anionic surfactants, such as sulfate-based surfactants, sulfonate-based surfactants, and phosphate-based surfactants; cationic surfactants, such as amine-salt-based surfactants and quaternary-ammonium-salt-based surfactants; and nonionic surfactants, such as polyethylene-glycol surfactants, alkylphenol-ethylene-

oxide-adduct-based surfactants, and polyhydric-alcohol-based surfactants. Among these surfactants, in particular, the anionic surfactants and the cationic surfactants may be used. The nonionic surfactants may be used in combination with the anionic surfactants and the cationic surfactants.

These surfactants may be used alone or in combination of two or more.

In the preparation of the resin particle dispersion liquid, the resin particles can be dispersed in a dispersion medium by any suitable dispersion method commonly used in the related art in which, for example, a rotary-shearing homogenizer, a ball mill, a sand mill, or a dyno mill that includes media is used. Depending on the type of the resin particles used, the resin particles may be dispersed in the dispersion medium by, for example, phase-inversion emulsification. Phase-inversion emulsification is a method in which the resin to be dispersed is dissolved in a hydrophobic organic solvent in which the resin is soluble, a base is added to the resulting organic continuous phase (i.e., O phase) to perform neutralization, and subsequently an aqueous medium (i.e., W phase) is charged in order to perform phase inversion from W/O to O/W and disperse the resin in the aqueous medium in the form of particles.

The volume-average diameter of the resin particles dispersed in the resin particle dispersion liquid is preferably, for example, 0.01  $\mu\text{m}$  or more and 1  $\mu\text{m}$  or less, is more preferably 0.08  $\mu\text{m}$  or more and 0.8  $\mu\text{m}$  or less, and is further preferably 0.1  $\mu\text{m}$  or more and 0.6  $\mu\text{m}$  or less.

The volume-average diameter of the resin particles is determined in the following manner. The particle diameter distribution of the resin particles is obtained using a laser-diffraction particle-size-distribution measurement apparatus (e.g., "LA-700" produced by HORIBA, Ltd.). The particle diameter distribution measured is divided into a number of particle diameter ranges (i.e., channels). For each range, in ascending order in terms of particle diameter, the cumulative volume is calculated and plotted to draw a cumulative distribution curve. A particle diameter at which the cumulative volume reaches 50% is considered to be the volume particle diameter D50v. The volume-average diameters of particles included in the other dispersion liquids are also determined in the above-described manner.

The content of the resin particles included in the resin particle dispersion liquid is preferably 5% by mass or more and 50% by mass or less and is more preferably 10% by mass or more and 40% by mass or less.

The colorant particle dispersion liquid, the release-agent particle dispersion liquid, and the like are also prepared as in the preparation of the resin particle dispersion liquid. In other words, the above-described specifications for the volume-average diameter of the particles included in the resin particle dispersion liquid, the dispersion medium of the resin particle dispersion liquid, the dispersion method used for preparing the resin particle dispersion liquid, and the content of the particles in the resin particle dispersion liquid can also be applied to colorant particles dispersed in the colorant particle dispersion liquid and release-agent particles dispersed in the release-agent particle dispersion liquid.

#### Aggregated Particle Formation Step

The resin particle dispersion liquid is mixed with the colorant particle dispersion liquid and the release-agent particle dispersion liquid.

In the resulting mixed dispersion liquid, heteroaggregation of the resin particles with the colorant particles and the release-agent particles is performed in order to form aggregated particles including the resin particles, the colorant

particles, and the release-agent particles, the aggregated particles having a diameter close to that of the desired toner particles.

Specifically, for example, a flocculant is added to the mixed dispersion liquid, and the pH of the mixed dispersion liquid is controlled to be acidic (e.g., pH of 2 or more and 5 or less). A dispersion stabilizer may be added to the mixed dispersion liquid as needed. Subsequently, the mixed dispersion liquid is heated to a temperature close to the glass transition temperature of the resin particles (specifically, e.g., [glass transition temperature of the resin particles—30° C.] or more and [the glass transition temperature—10° C.] or less), and thereby the particles dispersed in the mixed dispersion liquid are caused to aggregate together to form aggregated particles.

In the aggregated particle formation step, alternatively, for example, the above flocculant may be added to the mixed dispersion liquid at room temperature (e.g., 25° C.) while the mixed dispersion liquid is stirred using a rotary-shearing homogenizer. Then, the pH of the mixed dispersion liquid is controlled to be acidic (e.g., pH of 2 or more and 5 or less), and a dispersion stabilizer may be added to the mixed dispersion liquid as needed. Subsequently, the mixed dispersion liquid is heated in the above-described manner.

Examples of the flocculant include surfactants, inorganic metal salts, and divalent or higher metal complexes that have a polarity opposite to that of the surfactant included in the mixed dispersion liquid. Using a metal complex as a flocculant reduces the amount of surfactant used and, as a result, charging characteristics may be enhanced.

An additive capable of forming a complex or a bond similar to a complex with the metal ions contained in the flocculant may optionally be used in combination with the flocculant. An example of the additive is a chelating agent.

Examples of the inorganic metal salts include metal salts, such as calcium chloride, calcium nitrate, barium chloride, magnesium chloride, zinc chloride, aluminum chloride, and aluminum sulfate; and inorganic metal salt polymers, such as polyaluminum chloride, polyaluminum hydroxide, and calcium polysulfide.

The chelating agent may be a water-soluble chelating agent. Examples of such a chelating agent include oxycarboxylic acids, such as tartaric acid, citric acid, and gluconic acid; and aminocarboxylic acids, such as iminodiacetic acid (IDA), nitrilotriacetic acid (NTA), and ethylenediaminetetraacetic acid (EDTA).

The amount of the chelating agent used is preferably 0.01 parts by mass or more and 5.0 parts by mass or less and is more preferably 0.1 parts by mass or more and less than 3.0 parts by mass relative to 100 parts by mass of the resin particles.

#### Fusion-Coalescence Step

The aggregated particle dispersion liquid in which the aggregated particles are dispersed is heated to, for example, the glass transition temperature of the resin particles or more (e.g., temperature higher than the glass transition temperature of the resin particles by 10° C. to 30° C.) in order to perform fusion and coalescence of the aggregated particles. Hereby, toner particles are prepared.

The toner particles are prepared through the above-described steps.

It is also possible to prepare the toner particles by, after preparing the aggregated particle dispersion liquid in which the aggregated particles are dispersed, further mixing the aggregated particle dispersion liquid with a resin particle dispersion liquid in which resin particles are dispersed and subsequently performing aggregation such that the resin

## 15

particles are deposited on the surfaces of the aggregated particles in order to form second aggregated particles; and by heating the resulting second-aggregated particle dispersion liquid in which the second aggregated particles are dispersed and thereby causing fusion and coalescence of the second aggregated particles to occur in order to form toner particles having a core-shell structure.

After the completion of the fusion-coalescence step, the toner particles formed in the solution are subjected to any suitable cleaning step, solid-liquid separation step, and drying step that are known in the related art in order to obtain dried toner particles. In the cleaning step, the toner particles may be subjected to displacement washing using ion-exchange water to a sufficient degree from the viewpoint of electrification characteristics. Examples of a solid-liquid separation method used in the solid-liquid separation step include suction filtration and pressure filtration from the viewpoint of productivity. Examples of a drying method used in the drying step include freeze-drying, flash drying, fluidized drying, and vibrating fluidized drying from the viewpoint of productivity.

The toner according to the exemplary embodiment is produced by, for example, adding an external additive to the dried toner particles and mixing the resulting toner particles using a V-blender, a Henschel mixer, a Lodige mixer, or the like. Optionally, coarse toner particles may be removed using a vibrating screen classifier, a wind screen classifier, or the like.

## Electrostatic-Image Developer

An electrostatic-image developer according to the exemplary embodiment includes at least the toner according to the exemplary embodiment.

The electrostatic-image developer according to the exemplary embodiment may be a monocomponent developer including only the toner according to the exemplary embodiment or may be a two-component developer that is a mixture of the toner and a carrier.

The type of the carrier is not limited, and any suitable carrier known in the related art may be used. Examples of the carrier include a coated carrier prepared by coating the surfaces of cores including magnetic powder particles with a resin; a magnetic-powder-dispersed carrier prepared by dispersing and mixing magnetic powder particles in a matrix resin; and a resin-impregnated carrier prepared by impregnating a porous magnetic powder with a resin. The magnetic-powder-dispersed carrier and the resin-impregnated carrier may also be prepared by coating the surfaces of particles constituting the carrier, that is, core particles, with a resin.

Examples of the magnetic powder include powders of magnetic metals, such as iron, nickel, and cobalt; and powders of magnetic oxides, such as ferrite and magnetite.

Examples of the coat resin and the matrix resin include polyethylene, polypropylene, polystyrene, poly(vinyl acetate), poly(vinyl alcohol), poly(vinyl butyral), poly(vinyl chloride), poly(vinyl ether), poly(vinyl ketone), a vinyl chloride-vinyl acetate copolymer, a styrene-acrylic acid ester copolymer, a straight silicone resin including an organosiloxane bond and the modified products thereof, a fluorine resin, polyester, polycarbonate, a phenolic resin, and an epoxy resin. The coat resin and the matrix resin may optionally include additives, such as conductive particles. Examples of the conductive particles include particles of metals, such as gold, silver, and copper; and particles of carbon black, titanium oxide, zinc oxide, tin oxide, barium sulfate, aluminum borate, and potassium titanate.

## 16

The surfaces of the cores can be coated with a resin by, for example, using a coating-layer forming solution prepared by dissolving the coat resin and, as needed, various types of additives in a suitable solvent. The type of the solvent is not limited and may be selected with consideration of the type of the resin used, ease of applying the coating-layer forming solution, and the like.

Specific examples of a method for coating the surfaces of the cores with the coat resin include an immersion method in which the cores are immersed in the coating-layer forming solution; a spray method in which the coating-layer forming solution is sprayed onto the surfaces of the cores; a fluidized-bed method in which the coating-layer forming solution is sprayed onto the surfaces of the cores while the cores are floated using flowing air; and a kneader-coater method in which the cores of the carrier are mixed with the coating-layer forming solution in a kneader coater and subsequently the solvent is removed.

The mixing ratio (i.e., mass ratio) of the toner to the carrier in the two-component developer is preferably toner: carrier=1:100 to 30:100 and is more preferably 3:100 to 20:100.

## Image Forming Apparatus and Image Forming Method

An image forming apparatus according to the exemplary embodiment includes an image holding member; a charging unit that charges the surface of the image holding member; an electrostatic-image formation unit that forms an electrostatic image on the charged surface of the image holding member; a developing unit that includes an electrostatic-image developer and develops the electrostatic image formed on the surface of the image holding member with the electrostatic-image developer to form a toner image; a transfer unit that transfers the toner image formed on the surface of the image holding member onto the surface of a recording medium; a fixing unit that fixes the toner image onto the surface of the recording medium; and a cleaning unit that includes a blade arranged to come into contact with the surface of the image holding member and removes a toner that remains on the surface of the image holding member after transfer of the toner image with the blade.

An image forming apparatus according to the exemplary embodiment uses an image forming method (image forming method according to the exemplary embodiment) including charging the surface of the image holding member; forming an electrostatic image on the charged surface of the image holding member; developing the electrostatic image formed on the surface of the image holding member with the electrostatic-image developer according to the exemplary embodiment to form a toner image; transferring the toner image formed on the surface of the image holding member onto the surface of a recording medium; fixing the toner image onto the surface of the recording medium; and bringing a blade into contact with the surface of the image holding member after transfer of the toner image to remove a toner that remains on the surface of the image holding member.

The image forming apparatus according to the exemplary embodiment may be any image forming apparatus known in the related art, such as a direct-transfer image forming apparatus in which a toner image formed on the surface of an image holding member is directly transferred to a recording medium; an intermediate-transfer image forming apparatus in which a toner image formed on the surface of an image holding member is transferred onto the surface of an intermediate transfer body in the first transfer step and the toner image transferred on the surface of the intermediate transfer body is transferred onto the surface of a recording

medium in the second transfer step; and an image forming apparatus including a static-eliminating unit that eliminates static by irradiating the surface of an image holding member with static-eliminating light subsequent to the transfer of the toner image before the image holding member is again charged.

In the case where the image forming apparatus according to the exemplary embodiment is the intermediate-transfer image forming apparatus, the transfer unit may be constituted by, for example, an intermediate transfer body to which a toner image is transferred, a first transfer subunit that transfers a toner image formed on the surface of the image holding member onto the surface of the intermediate transfer body in the first transfer step, and a second transfer subunit that transfers the toner image transferred on the surface of the intermediate transfer body onto the surface of a recording medium in the second transfer step.

In the image forming apparatus according to the exemplary embodiment, for example, a portion including the developing unit may have a cartridge structure (i.e., process cartridge) detachably attachable to the image forming apparatus. An example of the process cartridge is a process cartridge including the electrostatic-image developer according to the exemplary embodiment and the developing unit.

An example of the image forming apparatus according to the exemplary embodiment is described below, but the image forming apparatus is not limited thereto. Hereinafter, only components illustrated in drawings are described; others are omitted.

FIG. 1 schematically illustrates the image forming apparatus according to the exemplary embodiment.

The image forming apparatus illustrated in FIG. 1 includes first to fourth electrophotographic image formation units **10Y**, **10M**, **10C**, and **10K** that form yellow (Y), magenta (M), cyan (C), and black (K) images, respectively, on the basis of color separation image data. The image formation units (hereinafter, referred to simply as "units") **10Y**, **10M**, **10C**, and **10K** are horizontally arranged in parallel at a predetermined distance from one another. The units **10Y**, **10M**, **10C**, and **10K** may be process cartridges detachably attachable to the image forming apparatus.

An intermediate transfer belt (example of the intermediate transfer body) **20** runs above and extends over the units **10Y**, **10M**, **10C**, and **10K**. The intermediate transfer belt **20** is wound around a drive roller **22** and a support roller **24** and runs clockwise in FIG. 1, that is, in the direction from the first unit **10Y** to the fourth unit **10K**. Using a spring or the like (not illustrated), a force is applied to the support roller **24** in a direction away from the drive roller **22**, thereby applying tension to the intermediate transfer belt **20** wound around the drive roller **22** and the support roller **24**. An intermediate transfer body-cleaning device **30** is disposed so as to come into contact with the image-carrier-side surface of the intermediate transfer belt **20** and to face the drive roller **22**.

Developing devices (examples of the developing units) **4Y**, **4M**, **4C**, and **4K** of the units **10Y**, **10M**, **10C**, and **10K** are supplied with yellow, magenta, cyan, and black toners stored in toner cartridges **8Y**, **8M**, **8C**, and **8K**, respectively.

Since the first to fourth units **10Y**, **10M**, **10C**, and **10K** have the same structure and the same action, the following description is made with reference to, as a representative, the first unit **10Y** that forms an yellow image and is located upstream in a direction in which the intermediate transfer belt runs.

The first unit **10Y** includes a photosensitive member **1Y** serving as an image holding member. The following components are disposed around the photosensitive member **1Y** sequentially in the counterclockwise direction: a charging roller (example of the charging unit) **2Y** that charges the surface of the photosensitive member **1Y** at a predetermined potential; an exposure device (example of the electrostatic-image formation unit) **3** that forms an electrostatic image by irradiating the charged surface of the photosensitive member **1Y** with a laser beam **3Y** based on a color separated image signal; a developing device (example of the developing unit) **4Y** that develops the electrostatic image by supplying a charged toner to the electrostatic image; a first transfer roller (example of the first transfer subunit) **5Y** that transfers the developed toner image to the intermediate transfer belt **20**; and a photosensitive-member cleaning device (example of the cleaning unit) **6Y** that removes a toner remaining on the surface of the photosensitive member **1Y** after the first transfer.

The photosensitive member cleaning device **6Y** includes a cleaning blade arranged to come into contact with the surface of the photosensitive member **1Y**. The cleaning blade is brought into contact with the surface of the photosensitive member **1Y** that keeps rotating after the transfer of the toner image and removes the toner particles remaining on the surface of the photosensitive member **1Y**.

The first transfer roller **5Y** is disposed so as to be in contact with the inner surface of the intermediate transfer belt **20** and to face the photosensitive member **1Y**. Each of the first transfer rollers **5Y**, **5M**, **5C**, and **5K** of the respective units is connected to a bias power supply (not illustrated) that applies a first transfer bias to the first transfer rollers. Each bias power supply varies the transfer bias applied to the corresponding first transfer roller on the basis of the control by a controller (not illustrated).

The action of forming a yellow image in the first unit **10Y** is described below.

Before the action starts, the surface of the photosensitive member **1Y** is charged at a potential of -600 to -800 V by the charging roller **2Y**.

The photosensitive member **1Y** is formed by stacking a photosensitive layer on a conductive substrate (e.g., volume resistivity at 20° C.:  $1 \times 10^{-6}$  Ωcm or less). The photosensitive layer is normally of high resistance (comparable with the resistance of ordinary resins), but, upon being irradiated with the laser beam, the specific resistance of the portion irradiated with the laser beam varies. Thus, the exposure device **3** irradiates the surface of the charged photosensitive member **1Y** with the laser beam **3Y** on the basis of the image data of the yellow image sent from the controller (not illustrated). As a result, an electrostatic image of yellow image pattern is formed on the surface of the photosensitive member **1Y**.

The term "electrostatic image" used herein refers to an image formed on the surface of the photosensitive member **1Y** by charging, the image being a "negative latent image" formed by irradiating a portion of the photosensitive layer with the laser beam **3Y** to reduce the specific resistance of the irradiated portion such that the charges on the irradiated surface of the photosensitive member **1Y** discharge while the charges on the portion that is not irradiated with the laser beam **3Y** remain.

The electrostatic image, which is formed on the photosensitive member **1Y** as described above, is sent to the predetermined developing position by the rotating photosensitive member **1Y**. The electrostatic image on the ph-

19

tosensitive member 1Y is developed and visualized in the form of a toner image by the developing device 4Y at the developing position.

The developing device 4Y includes an electrostatic-image developer including, for example, at least, a yellow toner and a carrier. The yellow toner is stirred in the developing device 4Y to be charged by friction and supported on a developer roller (example of the developer support), carrying an electric charge of the same polarity (i.e., negative) as the electric charge generated on the photosensitive member 1Y. The yellow toner is electrostatically adhered to the eliminated latent image portion on the surface of the photosensitive member 1Y as the surface of the photosensitive member 1Y passes through the developing device 4Y. Thus, the latent image is developed using the yellow toner. The photosensitive member 1Y on which the yellow toner image is formed keeps rotating at the predetermined rate, thereby transporting the toner image developed on the photosensitive member 1Y to the predetermined first transfer position.

Upon the yellow toner image on the photosensitive member 1Y reaching the first transfer position, first transfer bias is applied to the first transfer roller 5Y so as to generate an electrostatic force on the toner image in the direction from the photosensitive member 1Y toward the first transfer roller 5Y. Thus, the toner image on the photosensitive member 1Y is transferred to the intermediate transfer belt 20. The transfer bias applied has the opposite polarity (+) to that of the toner (-) and controlled to be, in the first unit 10Y, for example, +10  $\mu$ A by a controller (not illustrated).

After the transfer of the toner image, the photosensitive member 1Y keeps rotating and is brought into contact with the cleaning blade included in the photosensitive member cleaning device 6Y. The toner particles remaining on the photosensitive member 1Y are removed by the photosensitive-member cleaning device 6Y and then collected.

Each of the first transfer biases applied to first transfer rollers 5M, 5C, and 5K of the second, third, and fourth units 10M, 10C, and 10K is controlled in accordance with the first unit 10Y.

Thus, the intermediate transfer belt 20, on which the yellow toner image is transferred in the first unit 10Y, is successively transported through the second to fourth units 10M, 10C, and 10K while toner images of the respective colors are stacked on top of another.

The resulting intermediate transfer belt 20 on which toner images of four colors are multiple-transferred in the first to fourth units is then transported to a second transfer section including a support roller 24 being in contact with the inner surface of the intermediate transfer belt 20 and a second transfer roller (example of the second transfer subunit) 26 disposed on the image-carrier-side of the intermediate transfer belt 20. A recording paper (example of the recording medium) P is fed by a feed mechanism into a narrow space between the second transfer roller 26 and the intermediate transfer belt 20 that are brought into contact with each other at the predetermined timing. The second transfer bias is then applied to the support roller 24. The transfer bias applied here has the same polarity (-) as that of the toner (-) and generates an electrostatic force on the toner image in the direction from the intermediate transfer belt 20 toward the recording paper P. Thus, the toner image on the intermediate transfer belt 20 is transferred to the recording paper P. The intensity of the second transfer bias applied is determined on the basis of the resistance of the second transfer section which is detected by a resistance detector (not illustrated) that detects the resistance of the second transfer section and controlled by changing voltage.

20

Subsequently, the recording paper P is transported into a nip part of the fixing device (example of the fixing unit) 28 at which a pair of fixing rollers are brought into contact with each other. The toner image is fixed to the recording paper P to form a fixed image.

Examples of the recording paper P to which a toner image is transferred include plain paper used in electrophotographic copiers, printers, and the like. Instead of the recording paper P, OHP films and the like may be used as a recording medium.

The surface of the recording paper P may be smooth in order to enhance the smoothness of the surface of the fixed image. Examples of such a recording paper include coated paper produced by coating the surface of plain paper with resin or the like and art paper for printing.

The recording paper P, to which the color image has been fixed, is transported toward an exit portion. Thus, the series of the steps for forming a color image are terminated.

#### Process Cartridge and Toner Cartridge

20 A process cartridge according to the exemplary embodiment includes an image holding member, a developing unit that includes the electrostatic-image developer according to the exemplary embodiment and develops an electrostatic image formed on the surface of an image holding member with the electrostatic-image developer to form a toner image, and a cleaning unit that includes a blade arranged to come into contact with the surface of the image holding member and removes a toner that remains on the surface of the image holding member after transfer of the toner image with the blade. The process cartridge according to the exemplary embodiment is detachably attachable to an image forming apparatus.

The structure of the process cartridge according to the exemplary embodiment is not limited to the above-described one. The process cartridge according to the exemplary embodiment may include the developing unit and, as needed, at least one unit selected from a charging unit, an electrostatic-image formation unit, a transfer unit, and the like.

35 An example of the process cartridge according to the exemplary embodiment is described below, but the process cartridge is not limited thereto. Hereinafter, only components illustrated in FIG. 2 are described; others are omitted.

FIG. 2 schematically illustrates the process cartridge according to the exemplary embodiment.

40 A process cartridge 200 illustrated in FIG. 2 includes, for example, a photosensitive member 107 (example of the image holding member), a charging roller 108 (example of the charging unit) disposed on the periphery of the photosensitive member 107, a developing device 111 (example of the developing unit), and a photosensitive-member cleaning device 113 (example of the cleaning unit), which are combined into one unit using a housing 117 to form a cartridge. The housing 117 has an aperture 118 for exposure. A mounting rail 116 is disposed on the housing 117. The photosensitive-member cleaning device 113 includes a blade arranged to come into contact with the photosensitive member 107.

45 In FIG. 2, Reference numeral 109 denotes an exposure device (example of the electrostatic-image formation unit), Reference numeral 112 denotes a transfer device (example of the transfer unit), Reference numeral 115 denotes a fixing device (example of the fixing unit), and the Reference numeral 300 denotes recording paper (example of the recording medium).

50 A toner cartridge according to the exemplary embodiment is described below.

## 21

The toner cartridge according to the exemplary embodiment includes the toner according to the exemplary embodiment and is detachably attachable to an image forming apparatus. The toner cartridge includes a replacement toner that is to be supplied to the developing unit disposed inside an image forming apparatus.

The image forming apparatus illustrated in FIG. 1 is an image forming apparatus that includes the toner cartridges 8Y, 8M, 8C, and 8K detachably attached to the image forming apparatus. Each of the developing devices 4Y, 4M, 4C, and 4K is connected to a specific one of the toner cartridges which corresponds to the developing device (color) with a toner feed pipe (not illustrated). When the amount of toner contained in a toner cartridge is small, the toner cartridge is replaced.

## EXAMPLES

Details of the exemplary embodiment of the present disclosure are described below with reference to Examples below. The exemplary embodiment of the present disclosure is not limited to Examples below. Hereinafter, the terms "part" and "%" are on a mass basis unless otherwise specified.

## Preparation of Toner Particles

## Preparation of Amorphous Polyester Resin Dispersion Liquid (A1)

Terephthalic acid: 70 parts

Fumaric acid: 30 parts

Ethylene glycol: 44 parts

1,5-Pentanediol: 46 parts

Into a flask equipped with a stirring device, a nitrogen introducing tube, a temperature sensor, and a fractionating column, the above materials are charged. Under a nitrogen stream, the temperature is increased to 210° C. over 1 hour, and 1 part of titanium tetraethoxide relative to 100 parts of the total amount of the above materials is added to the flask. While the product water is removed by distillation, the temperature is increased to 240° C. over 0.5 hours and dehydration condensation is continued for 1 hour at 240° C. Subsequently, the product of the reaction is cooled. Hereby, an amorphous polyester resin having a weight-average molecular weight of 94,500 and a glass transition temperature of 61° C. is prepared.

Into a container equipped with a temperature control unit and a nitrogen purging unit, 40 parts of ethyl acetate and 25 parts of 2-butanol are charged to form a mixed solvent. To the mixed solvent, 100 parts of the amorphous polyester resin is gradually added and dissolved in the mixed solvent. To the resulting solution, a 10% aqueous ammonia solution is added in an amount 3 times by mole with respect to the acid value of the resin. The resulting mixture is stirred for 30 minutes. Then, the inside of the container is purged with dry nitrogen. While the temperature is maintained to be 40° C. and the liquid mixture is stirred, 400 parts of ion-exchange water is added dropwise to the container in order to perform emulsification. After the addition of ion-exchange water has been terminated, the resulting emulsion is cooled to 25° C. Hereby, a resin particle dispersion liquid that includes resin particles having a volume-average particle size of 210 nm dispersed therein is prepared. Ion-exchange water is added to the resin particle dispersion liquid to adjust the solid content in the dispersion liquid to be 20%. Hereby, an amorphous polyester resin dispersion liquid (A1) is prepared. Preparation of Crystalline Polyester Resin Dispersion Liquid (B1)

## 22

Dimethyl sebacate: 97 parts  
Sodium dimethyl-5-sulfonate isophthalate: 3 parts  
Ethylene glycol: 100 parts  
Dibutyltin oxide (catalyst): 0.3 parts

The above materials are charged into a three-necked flask dried by heating. Subsequently, the atmosphere inside the three-necked flask is replaced with an inert atmosphere by purging with a nitrogen gas. The resulting mixture is stirred by mechanical stirring and caused to reflux at 180° C. for 5 hours. Then, the temperature is gradually increased to 240° C. under reduced pressure and stirring is performed for 2 hours. When the mixture becomes viscous, air cooling is performed and the reaction is stopped. Hereby, a crystalline polyester resin having a weight-average molecular weight of 9,700 and a melting temperature of 84° C. is prepared.

Then, 90 parts of the crystalline polyester resin, 1.8 parts of an anionic surfactant "Neogen RK" produced by DKS Co. Ltd., and 210 parts of ion-exchange water are mixed with one another. The resulting mixture is heated to 100° C. and dispersed with a homogenizer "ULTRA-TURRAX T50" produced by IKA. Subsequently, a dispersion treatment is performed for 1 hour using a pressure-discharge Gaulin homogenizer. Hereby, a resin particle dispersion liquid that includes resin particles having a volume-average particle size of 205 nm dispersed therein is prepared. Ion-exchange water is added to the resin particle dispersion liquid in order to adjust the solid content in the dispersion liquid to be 20%. Hereby, a crystalline polyester resin dispersion liquid (B1) is prepared.

## Preparation of Release Agent Particle Dispersion Liquid (W1)

Paraffin wax "HNP-9" produced by Nippon Seiro Co., Ltd.: 100 parts

Anionic surfactant "Neogen RK" produced by Dai-ichi Kogyo Seiyaku Co., Ltd.: 1 part

Ion-exchange water: 350 parts

The above materials are mixed with one another and heated to 100° C. The resulting mixture is dispersed with a homogenizer "ULTRA-TURRAX T50" produced by IKA and then further dispersed with a pressure-discharge Gaulin homogenizer. Hereby, a release agent particle dispersion liquid in which release agent particles having a volume-average particle size of 200 nm are dispersed is prepared. Ion-exchange water is added to the release agent particle dispersion liquid in order to adjust the solid content in the dispersion liquid to be 20%. Hereby, a release agent particle dispersion liquid (W1) is prepared.

## Preparation of Colorant Particle Dispersion Liquid (K1)

Carbon black "Regal330" produced by Cabot Corporation: 50 parts

Ionic surfactant "Neogen RK" produced by DKS Co. Ltd.: 5 parts

Ion-exchange water: 195 parts

The above materials are mixed with one another, and the resulting mixture is dispersed with Ultimizer produced by Sugino Machine Limited at 240 MPa for 10 minutes. Hereby, a colorant particle dispersion liquid (K1) having a solid content of 20% is prepared.

## Preparation of Toner Particles

Ion-exchange water: 200 parts

Amorphous polyester resin dispersion liquid (A1): 150 parts

Crystalline polyester resin dispersion liquid (B1): 10 parts  
Release agent particle dispersion liquid (W1): 10 parts

Colorant particle dispersion liquid (K1): 15 parts

Anionic surfactant (TaycaPower): 2.8 parts

The above materials are charged into a round-bottom flask made of stainless steel. After the pH has been adjusted to be

3.5 by addition of 0.1 N nitric acid, an aqueous polyaluminum chloride solution prepared by dissolving 2 parts of polyaluminum chloride (30% powder produced by Oji Paper Co., Ltd.) in 30 parts of ion-exchange water is added to the flask. After dispersion has been performed with a homogenizer "ULTRA-TURRAX T50" produced by IKA at 30° C., the temperature is increased to 45° C. in a heating oil bath. Then, holding is performed until the volume-average particle size reaches 4.9  $\mu\text{m}$ . Subsequently, 60 parts of the amorphous polyester resin dispersion liquid (A1) is added to the flask and holding is performed for 30 minutes. When the volume-average particle size reaches 5.2  $\mu\text{m}$ , another 60 parts of the amorphous polyester resin dispersion liquid (A1) is added to the flask and holding is performed for 30 minutes. Then, 20 parts of a 10%, aqueous solution of nitrilotriacetic acid (NTA) metal salt "Chelest 70" produced by Chelest Corporation is added to the flask. Subsequently, the pH is adjusted to be 9.0 by addition of a 1 N aqueous sodium hydroxide solution. Then, 1 part of an anionic surfactant "TaycaPower" is added to the flask. While stirring is continued, the temperature is increased to 85° C. and then holding is performed for 5 hours. Subsequently, the temperature is reduced to 20° C. at a rate of 20° C./min. Then, filtration is performed. The resulting substance is sufficiently washed with ion-exchange water and dried to form toner particles (1) having a volume-average particle size of 5.7  $\mu\text{m}$  and an average circularity of 0.971.

#### Preparation of Layered Compound Particles

#### Preparation of Melamine Cyanurate Particles

A commercial melamine cyanurate "MC-4500" produced by Nissan Chemical Corporation is disintegrated and classified with a jet mill to prepare the melamine cyanurate particles (1) to (5) described below. In Table 1, "MC" means melamine cyanurate.

Melamine cyanurate particles (1): volume-average particle size: 1.0  $\mu\text{m}$

Melamine cyanurate particles (2): volume-average particle size: 3.5  $\mu\text{m}$

Melamine cyanurate particles (3): volume-average particle size: 2.9  $\mu\text{m}$

Melamine cyanurate particles (4): volume-average particle size: 0.4  $\mu\text{m}$

Melamine cyanurate particles (5): volume-average particle size: 0.2  $\mu\text{m}$

#### Preparation of Boron Nitride Particles

Commercial boron nitride particles "AP-10S" produced by MARUKA are prepared. The boron nitride particles have a volume-average particle size of 2.4  $\mu\text{m}$ . In Table 1, "BN" means boron nitride.

#### Preparation of Oil-Treated Particles

#### Preparation of Silicone Oil-Treated Silica Particles (1)

$\text{SiCl}_4$ , a hydrogen gas, and an oxygen gas are mixed with one another in a mixing chamber of a firing burner. The resulting mixture is burnt at 1,000° C. or more and 3,000° C. or less. A silica powder is collected from the burnt gas. Hereby, silica particles (1) are prepared. The volume-average particle size (D50v) of the silica particles (1) is adjusted to be 65 nm by setting the molar ratio between the hydrogen gas and the oxygen gas to be 1.38:1.

Into an evaporator, 100 parts of the silica particles (1) and 500 parts of ethanol are charged. The resulting mixture is stirred for 15 minutes while the temperature is maintained to be 40° C. Subsequently, 15 parts of a dimethyl silicone oil is charged into the evaporator and stirring is performed for 15 minutes. Another 15 parts of a dimethyl silicone oil is charged into the evaporator and stirring is performed for 15 minutes. Then, the temperature is increased to 90° C., and

ethanol is removed by drying under reduced pressure. Subsequently, vacuum drying is performed at 120° C. for 30 minutes. Hereby, silicone oil-treated silica particles (1) having a volume-average particle size of 65 nm and a free oil content of 1.5% are prepared. Preparation of Silicone Oil-Treated Silica Particles (2)

Silicone oil-treated silica particles (2) having a volume-average particle size of 65 nm and a free oil content of 6.0% are prepared as in the preparation of the silicone oil-treated silica particles (1), except that the amount of the dimethyl silicone oil used for the first time is changed to 20 parts, and the amount of the dimethyl silicone oil used for the second time is changed to 30 parts.

#### Preparation of Silicone Oil-Treated Silica Particles (3)

Silicone oil-treated silica particles (3) having a volume-average particle size of 65 nm and a free oil content of 5.0% are prepared as in the preparation of the silicone oil-treated silica particles (1), except that the amount of the dimethyl silicone oil used for the first time is changed to 20 parts, and the amount of the dimethyl silicone oil used for the second time is changed to 25 parts.

#### Preparation of Silicone Oil-Treated Silica Particles (4)

Silicone oil-treated silica particles (4) having a volume-average particle size of 65 nm and a free oil content of 4.4% are prepared as in the preparation of the silicone oil-treated silica particles (1), except that the amount of the dimethyl silicone oil used for the first time is changed to 20 parts, and the amount of the dimethyl silicone oil used for the second time is changed to 22 parts.

#### Preparation of Silicone Oil-Treated Silica Particles (5)

Silicone oil-treated silica particles (5) having a volume-average particle size of 65 nm and a free oil content of 2.5% are prepared as in the preparation of the silicone oil-treated silica particles (1), except that the amount of the dimethyl silicone oil used for the first time is changed to 20 parts, and the amount of the dimethyl silicone oil used for the second time is changed to 20 parts.

#### Preparation of Silicone Oil-Treated Silica Particles (6)

Silicone oil-treated silica particles (6) having a volume-average particle size of 65 nm and a free oil content of 2.0% are prepared as in the preparation of the silicone oil-treated silica particles (1), except that the amount of the dimethyl silicone oil used for the first time is changed to 15 parts, and the amount of the dimethyl silicone oil used for the second time is changed to 20 parts.

#### Preparation of Silicone Oil-Treated Silica Particles (7)

Silicone oil-treated silica particles (7) having a volume-average particle size of 65 nm and a free oil content of 1.25% are prepared as in the preparation of the silicone oil-treated silica particles (1), except that the amount of the dimethyl silicone oil used for the first time is changed to 10 parts, and the amount of the dimethyl silicone oil used for the second time is changed to 10 parts.

#### Preparation of Silicone Oil-Treated Silica Particles (8)

Silicone oil-treated silica particles (8) having a volume-average particle size of 65 nm and a free oil content of 0.25% are prepared as in the preparation of the silicone oil-treated silica particles (1), except that the amount of the dimethyl silicone oil used for the first time is changed to 1 part, and the amount of the dimethyl silicone oil used for the second time is changed to 1 part.

#### Preparation of Silicone Oil-Treated PMMA Particles

While 100 parts of polymethyl methacrylate (PMMA) particles having a volume-average particle size (D50v) of 300 nm are stirred and the temperature is maintained to be 60° C., a solution containing 20 parts of a dimethyl silicone oil having a weight-average molecular weight of 12,100 and

a number-average molecular weight of 2,030 and 20 parts of hexane is sprayed to the PMMA particles. Subsequently, the solvent is removed by drying while stirring is performed.

Then, while stirring is performed, the temperature is increased to 300° C. and holding is performed at 300° C. for 1 hour. Hereby, silicone oil-treated PMMA particles having a volume-average particle size of 300 nm and a free oil content of 1.5% are prepared.

#### Preparation of Carrier

After 500 parts of spherical magnetite powder particles having a volume-average particle size of 0.55  $\mu\text{m}$  have been stirred with a Henschel mixer, 5 parts of a titanate coupling agent is added. Then, temperature is increased to 100° C. and stirring is performed for 30 minutes. Subsequently, 6.25 parts of phenol, 9.25 parts of 35% formalin, 500 parts of the magnetite particles treated with a titanate coupling agent, 6.25 parts of 25% ammonia water, and 425 parts of water are charged into a four-necked flask. While the resulting mixture is stirred, the reaction is conducted at 85° C. for 120 minutes. Then, the temperature is reduced to 25° C. After 500 parts of water has been added to the flask, the resulting supernatant is removed and the precipitate is washed with water. The precipitate is dried by heating under reduced pressure to form a carrier having an average particle size of 35  $\mu\text{m}$ .

#### Example 1

The toner particles (1), the melamine cyanurate particles (1), and the silicone oil-treated silica particles (1) are charged into a sample mill at the proportions described in Table 1. The resulting mixture is stirred at 10,000 rpm for 30 seconds. Subsequently, screening is performed with a vibration sieve having an opening of 45  $\mu\text{m}$ . Hereby, a toner having a volume-average particle size of 5.7  $\mu\text{m}$  is prepared. The toner and the carrier are charged into a V-blender at a mass ratio of Toner:Carrier=5:95. The resulting mixture is stirred for 20 minutes to form a developer.

#### Examples 2 to 9

Toners and developers are prepared as in Example 1, except that the amount of the melamine cyanurate particles (1) used or the type and amount of the oil-treated particles used are changed.

#### Examples 10 to 15

Toners and developers are prepared as in Example 1, except that the type of the layered compound particles used or the type of the oil-treated particles used are changed.

#### Comparative Examples 1 and 2

Toners and developers are prepared as in Example 1, except that the amount of the melamine cyanurate particles (1) used and the type and amount of the oil-treated particles used are changed.

#### Performance Evaluations

Colored Streaks Formed when Image is Continuously Formed in Low-Temperature Low-Humidity Environment (Colored Streaks Due to Slip-Through of Toner)

An image having an area coverage of 0.2% is formed on 100,000 A4 size paper sheets with a modification of "700 Digital Color Press" produced by Fuji Xerox Co., Ltd. at 10° C. and a relative humidity of 10%. Subsequently, an image chart that is a combination of a solid image and a halftone image having a toner deposition density of 0.1 mg/cm<sup>2</sup> is formed on 500 A4 size paper sheets. The 10th, 50th, 100th, and 500th paper sheets are visually inspected and the total number of the colored streaks formed in the halftone images is counted and classified in the following manner.

G1: The number of the colored streaks is 0.

G2: The number of the colored streaks is 1.

G3: The number of the colored streaks is 2 to 5; acceptable.

G4: The number of the colored streaks is 6 or more; not acceptable in the practical use.

Colored Streaks Formed when Image is Continuously Formed in High-Temperature High-Humidity Environment (Colored Streaks Due to Wearing of Blade)

An image having an area coverage of 0.2% is formed on 100,000 sheets with a modification of "700 Digital Color Press" produced by Fuji Xerox Co., Ltd. at 28° C. and a relative humidity of 85%. Subsequently, an image chart that is a combination of a solid image and a halftone image having a toner deposition density of 0.1 mg/cm<sup>2</sup> is formed on an A4 size paper sheet. The halftone image is visually inspected, and the butting portion of the cleaning blade is observed with a microscope "VH6200" produced by Keyence Corporation at a 100-fold magnification. The number of the colored streaks formed in the halftone image and the condition of the butting portion of the cleaning blade are classified in the following manner.

G1: The number of the colored streaks is 0, and chipping of the cleaning blade is not observed.

G2: The number of the colored streaks is 0, and chipping of the cleaning blade is observed.

G3: The number of the colored streaks is 1 to 5, and chipping of the cleaning blade is observed; acceptable.

G4: The number of the colored streaks is 6 or more, and chipping of the cleaning blade is observed; not acceptable in the practical use.

TABLE 1

|                       | Layered compound particles |          |                                                |                                     | Oil-treated particles |          |                                   |                           |
|-----------------------|----------------------------|----------|------------------------------------------------|-------------------------------------|-----------------------|----------|-----------------------------------|---------------------------|
|                       | Type                       | Compound | Volume-average particle size ( $\mu\text{m}$ ) | Content in entire toner Ma (mass %) | Type                  | Compound | Volume-average particle size (nm) | Free oil content (mass %) |
|                       |                            |          |                                                |                                     |                       |          |                                   |                           |
| Comparative example 1 | (1)                        | MC       | 1.0                                            | 1.1                                 | (7)                   | Silica   | 65                                | 1.25                      |
| Comparative example 2 | (1)                        | MC       | 1.0                                            | 0.008                               | (3)                   | Silica   | 65                                | 5.0                       |
| Example 1             | (1)                        | MC       | 1.0                                            | 0.1                                 | (1)                   | Silica   | 65                                | 1.5                       |
| Example 2             | (1)                        | MC       | 1.0                                            | 0.01                                | (3)                   | Silica   | 65                                | 5.0                       |
| Example 3             | (1)                        | MC       | 1.0                                            | 0.01                                | (4)                   | Silica   | 65                                | 4.4                       |
| Example 4             | (1)                        | MC       | 1.0                                            | 0.1                                 | (2)                   | Silica   | 65                                | 6.0                       |

TABLE 1-continued

|            | (1) MC | 1.0 | 0.1 | (3) Silica | 65  | 5.0  | 4   | Performance evaluations |    |      |   |
|------------|--------|-----|-----|------------|-----|------|-----|-------------------------|----|------|---|
|            |        |     |     |            |     |      |     | (8) Silica              | 65 | 0.25 | 2 |
| Example 5  | (1) MC | 1.0 | 0.1 | (8) Silica | 65  | 0.25 | 1   |                         |    |      |   |
| Example 6  | (1) MC | 1.0 | 0.1 | (8) Silica | 65  | 0.25 | 1   |                         |    |      |   |
| Example 7  | (1) MC | 1.0 | 0.1 | (8) Silica | 65  | 0.25 | 1   |                         |    |      |   |
| Example 8  | (1) MC | 1.0 | 1   | (6) Silica | 65  | 2.0  | 0.5 |                         |    |      |   |
| Example 9  | (1) MC | 1.0 | 1   | (5) Silica | 65  | 2.5  | 0.4 |                         |    |      |   |
| Example 10 | (2) MC | 3.5 | 0.1 | (1) Silica | 65  | 1.5  | 2   |                         |    |      |   |
| Example 11 | (3) MC | 2.9 | 0.1 | (1) Silica | 65  | 1.5  | 2   |                         |    |      |   |
| Example 12 | (4) MC | 0.4 | 0.1 | (1) Silica | 65  | 1.5  | 2   |                         |    |      |   |
| Example 13 | (5) MC | 0.2 | 0.1 | (1) Silica | 65  | 1.5  | 2   |                         |    |      |   |
| Example 14 | (1) MC | 1.0 | 0.1 | PMMA       | 300 | 1.5  | 2   |                         |    |      |   |
| Example 15 | BN     | 2.4 | 0.1 | (1) Silica | 65  | 1.5  | 2   |                         |    |      |   |

  

|                       | Free oil content in entire toner | Content ratio | Content ratio | Colored streaks                                      |                                                   |                                                                      |
|-----------------------|----------------------------------|---------------|---------------|------------------------------------------------------|---------------------------------------------------|----------------------------------------------------------------------|
|                       |                                  |               |               | low-temperature low-humidity (slip-through of toner) | high-temperature high-humidity (wearing of blade) | Colored streaks in high-temperature high-humidity (wearing of blade) |
| Comparative example 1 | 0.01                             | 110           | 0.7           | G4                                                   | G1                                                |                                                                      |
| Comparative example 2 | 0.2                              | 0.04          | 500           | G1                                                   | G4                                                |                                                                      |
| Example 1             | 0.03                             | 3.3           | 20            | G1                                                   | G1                                                |                                                                      |
| Example 2             | 0.2                              | 0.05          | 400           | G1                                                   | G3                                                |                                                                      |
| Example 3             | 0.2                              | 0.05          | 450           | G1                                                   | G3                                                |                                                                      |
| Example 4             | 0.24                             | 0.4           | 40            | G1                                                   | G2                                                |                                                                      |
| Example 5             | 0.2                              | 0.5           | 40            | G1                                                   | G2                                                |                                                                      |
| Example 6             | 0.005                            | 20            | 20            | G2                                                   | G1                                                |                                                                      |
| Example 7             | 0.0025                           | 40            | 10            | G2                                                   | G1                                                |                                                                      |
| Example 8             | 0.01                             | 100           | 0.5           | G3                                                   | G1                                                |                                                                      |
| Example 9             | 0.01                             | 100           | 0.4           | G3                                                   | G1                                                |                                                                      |
| Example 10            | 0.03                             | 3.3           | 20            | G3                                                   | G1                                                |                                                                      |
| Example 11            | 0.03                             | 3.3           | 20            | G2                                                   | G1                                                |                                                                      |
| Example 12            | 0.03                             | 3.3           | 20            | G1                                                   | G2                                                |                                                                      |
| Example 13            | 0.03                             | 3.3           | 20            | G1                                                   | G3                                                |                                                                      |
| Example 14            | 0.03                             | 3.3           | 20            | G2                                                   | G2                                                |                                                                      |
| Example 15            | 0.03                             | 3.3           | 20            | G2                                                   | G2                                                |                                                                      |

The foregoing description of the exemplary embodiment of the present disclosure has been provided for the purposes of illustration and description. It is not intended to be exhaustive or to limit the disclosure to the precise forms disclosed. Obviously, many modifications and variations will be apparent to practitioners skilled in the art. The embodiment was chosen and described in order to best explain the principles of the disclosure and its practical applications, thereby enabling others skilled in the art to understand the disclosure for various embodiments and with the various modifications as are suited to the particular use contemplated. It is intended that the scope of the disclosure be defined by the following claims and their equivalents.

What is claimed is:

- An electrostatic-image developing toner comprising: toner particles; layered compound particles; and a free oil, wherein a mass ratio Ma/Mb of a content Ma of the layered compound particles to a content Mb of the free oil is 0.05 or more and 100 or less, and the layered compound particles include at least one type of particles selected from the group consisting of melamine cyanurate particles, boron nitride particles, and graphite fluoride particles.
- The electrostatic-image developing toner according to claim 1, wherein the content of the free oil is 0.005% by mass or more and 0.2% by mass or less of a total amount of the electrostatic-image developing toner.

- The electrostatic-image developing toner according to claim 2, wherein the layered compound particles have a volume-average particle size of 0.4  $\mu\text{m}$  or more and less than 3.0  $\mu\text{m}$ .
- The electrostatic-image developing toner according to claim 3, wherein the mass ratio Ma/Mb of the content Ma of the layered compound particles to the content Mb of the free oil is 0.2 or more and 100 or less.
- The electrostatic-image developing toner according to claim 2, wherein the mass ratio Ma/Mb of the content Ma of the layered compound particles to the content Mb of the free oil is 0.2 or more and 100 or less.
- The electrostatic-image developing toner according to claim 2, wherein the content of the free oil is 0.01% by mass or more and 0.12% by mass or less of the total amount of the electrostatic-image developing toner.
- The electrostatic-image developing toner according to claim 1, wherein the layered compound particles have a volume-average particle size of 0.4  $\mu\text{m}$  or more and less than 3.0  $\mu\text{m}$ .
- The electrostatic-image developing toner according to claim 7, wherein the mass ratio Ma/Mb of the content Ma of the layered compound particles to the content Mb of the free oil is 0.2 or more and 100 or less.

29

9. The electrostatic-image developing toner according to claim 7,

wherein the volume-average particle size of the layered compound particles is 0.5  $\mu\text{m}$  or more and 2.5  $\mu\text{m}$  or less.

10. The electrostatic-image developing toner according to claim 1,

wherein the mass ratio Ma/Mb of the content Ma of the layered compound particles to the content Mb of the free oil is 0.2 or more and 100 or less.

11. The electrostatic-image developing toner according to claim 1, further comprising particles treated with an oil.

12. The electrostatic-image developing toner according to claim 11,

wherein the particles treated with an oil include silica particles treated with an oil.

13. The electrostatic-image developing toner according to claim 11,

wherein a mass ratio Mc/Ma of a content Mc of the particles treated with an oil to the content Ma of the layered compound particles is 0.5 or more and 400 or less.

14. The electrostatic-image developing toner according to claim 13,

wherein the mass ratio Mc/Ma of the content Mc of the particles treated with an oil to the content Ma of the layered compound particles is 0.5 or more and 200 or less.

15. The electrostatic-image developing toner according to claim 1,

wherein the layered compound particles include at least one type of melamine cyanurate particles.

16. An electrostatic-image developer comprising the electrostatic-image developing toner according to claim 1.

17. A process cartridge detachably attachable to an image forming apparatus, the process cartridge comprising:

an image holding member;  
a developing unit that includes the electrostatic-image developer according to claim 16 and develops an electrostatic image formed on a surface of the image holding member with the electrostatic-image developer to form a toner image; and

a cleaning unit that includes a blade arranged to come into contact with the surface of the image holding member

30

and removes a toner that remains on the surface of the image holding member after transfer of the toner image with the blade.

18. An image forming apparatus comprising:  
an image holding member;

a charging unit that charges a surface of the image holding member;  
an electrostatic-image formation unit that forms an electrostatic image on the charged surface of the image holding member;

a developing unit that includes the electrostatic-image developer according to claim 16 and develops the electrostatic image formed on the surface of the image holding member with the electrostatic-image developer to form a toner image;

a transfer unit that transfers the toner image formed on the surface of the image holding member onto a surface of a recording medium;

a fixing unit that fixes the toner image transferred on the surface of the recording medium; and

a cleaning unit that includes a blade arranged to come into contact with the surface of the image holding member and removes a toner that remains on the surface of the image holding member after transfer of the toner image with the blade.

19. An image forming method comprising:  
charging a surface of an image holding member;

forming an electrostatic image on the charged surface of the image holding member;

developing the electrostatic image formed on the surface of the image holding member with the electrostatic-image developer according to claim 16 to form a toner image;

transferring the toner image formed on the surface of the image holding member onto a surface of a recording medium;

fixing the toner image transferred on the surface of the recording medium; and

bringing a blade into contact with the surface of the image holding member after transfer of the toner image to remove a toner that remains on the surface of the image holding member.

20. A toner cartridge detachably attachable to an image forming apparatus, the toner cartridge comprising the electrostatic-image developing toner according to claim 1.

\* \* \* \* \*